

## UNITED STATES PATENT OFFICE

2,085,137

## ABRASIVE ARTICLE

Charles E. Wooddell and John F. Barnes, Niagara Falls, N. Y., assignors, by mesne assignments, to The Carborundum Company, Niagara Falls, N. Y., a corporation of Delaware

No Drawing. Application December 8, 1933,  
Serial No. 701,532

9 Claims. (Cl. 51—278)

This invention relates to an improvement in the manufacture of abrasive articles and consists in producing such articles having a porous or cellular structure.

5 Abrasive articles, for example, grinding wheels, are, in general, made from graded abrasive grains mixed with bonding materials. This mixture is moistened with water, formed into the desired shape, dried and burned in a kiln. It 10 has been the practice to control the porosity of the article within a limited range of variation, by varying the grain size of the abrasive material, by varying the percentage of bond used, by the pressure applied during the forming, by the 15 addition of wood flour which burns out leaving pore spaces, or by other changes.

The present invention contemplates close control of the porosity and cell structure of finished abrasive articles by adding to the mix of granulated abrasive material and bond, granulated, oxidizable, non-compressible material which will burn away during the firing of the article in the kiln leaving pores of a number and character depending on the relative quantity and size of the oxidizable, non-compressible material used.

20 An object of this invention, therefore, is to provide a method of making abrasive articles of a predetermined porosity and having pores or interstices of a predetermined size.

30 Another object is to provide a mix from which abrasive articles having the desired characteristics as to porosity and cell structure may be made.

Other objects of the invention will be apparent from the following description and appended 35 claims.

The granulated material added to the mix as set forth above may be any suitable material which will not be compressed in the mix by the pressure used to form the abrasive articles and 40 which will burn away during the firing of the articles in the kiln for example coke.

The granulated coke used may be mulled or not mulled as found desirable in use. If used directly as crushed and graded it will have very 45 irregular shapes with many sharp points and edges. If mulled, e. g., put through a slow revolving ball mill, the sharp corners and edges will be worn off and the granules will be more rounded in shape and contour.

50 Any coke or related material, such as charcoal, may be used in carrying out the present invention, but for best results petroleum coke will be found desirable since it is relatively free from ash which might alter the character of the bond.

55 Depending upon the cellular structure desired

in the finished abrasive article the size of the granular coke may be smaller than, larger than, or equal to, that of the granular abrasive material used in the mix. For grinding many materials it may be necessary to have a highly porous article having a great number of pores or interstices substantially equal to, or smaller than, the abrasive grains. To produce such an article it is desirable to use in the mix coke grains smaller than or substantially equal to the abrasive grains. 10 in size. This does not mean, however, that the size of the pores in the finished article is equal to the size of the coke grains used, as the size of the pores is affected by other factors such as the nature and quantity of the bond used and the 15 degree of compression reached in forming the article. By controlling these factors as well as the size of the coke grains the cellular structure of the finished article may be determined in advance.

20 When coke smaller than, or substantially the same size as the abrasive material is used, each abrasive grain in the finished article will contact with practically all the adjacent grains as in the present non-porous articles, except that at 25 intervals varying in frequency as the degree of porosity desired, several grains will be so spaced as to provide a void or interstice larger than those formed by the vitrification of the bond but not substantially larger than each of the adjacent 30 grains of abrasive.

For grinding other material it may be necessary to have an abrasive article wherein there are relatively large pores, compared to the size of the abrasive grains. The pores of such an 35 article may be many times the size of the abrasive grains so that the walls of the pores are formed of a large number of abrasive grains. For the production of such articles it is necessary to add to the mix coke particles substantially 40 equal to or larger than the abrasive grains. For example, to produce an abrasive article having pores many times the size of the abrasive grains it is necessary to use coke grains many times the size of the abrasive particles.

45 When coke is granulated the particles or granules formed take very irregular and different shapes. When these particles are mixed in the abrasive article and subsequently burned out during the firing of the article the voids or interstices will in general take on substantially the 50 shape of the particles of coke previously located therein.

The proportion of granulated coke used in the mix is determined by the degree of porosity de- 55

sired in the finished product. The amount may be as large as is practicable to produce a porous article which is also strong enough for the use for which it is intended. In preparing articles for most purposes the proportion of coke used is 5 to 30 percent by weight of the abrasive and bond used.

As an illustration of the invention a mix having the following formula may be prepared and used to produce a porous abrasive article:

| Parts by weight             |    |
|-----------------------------|----|
| Abrasive grain (80 grit)    | 85 |
| Vitreous bond (through 109) | 15 |
| Calcined coke (40 on 74)    | 15 |
| Temporary binder            | 2  |

It will be noted that the coke used in the above example is larger in grain size than the abrasive grains. This mix will, therefore, when properly pressed into shape and burned, produce a porous abrasive article having pores several times the size of the abrasive grains. By using abrasive grains and coke of equal grain size and in the same proportion by weight as above, an equally porous article having relatively smaller pores may be produced. For example, the following formula could be used to produce an article having pores substantially the same size as the abrasive grains:

| Parts by weight                  |    |
|----------------------------------|----|
| Abrasive grain (40 grit)         | 85 |
| Vitreous bond (through 109)      | 15 |
| Calcined coke (through 40 on 74) | 20 |
| Temporary binder                 | 2  |

To produce an article having pores smaller than the abrasive grains the following formula could be used:

| Parts by weight                   |    |
|-----------------------------------|----|
| Abrasive grain (40 grit)          | 85 |
| Vitreous bond (through 109)       | 15 |
| Calcined coke (through 74 on 150) | 20 |
| Temporary binder                  | 2  |

The following formula could be used to produce an article having pores many times the size of the abrasive grains used:

| Parts by weight                  |    |
|----------------------------------|----|
| Abrasive grain (150 grit)        | 80 |
| Vitreous bond (through 109)      | 20 |
| Calcined coke (through 40 on 74) | 20 |
| Temporary binder                 | 2  |

By means of the present invention it is possible to economically produce abrasive articles having any practicable number and shape of cells. Articles which are light in weight and yet possess sufficient internal strength may be so produced. Because the use of coke increases the porosity and tends to spread out the abrasive grains a relatively large proportion of bond may be used, maintaining or increasing the internal strength, without increasing the tendency of the article to glaze in use. The use of coke or similar material is advantageous in that it is not compressed by the pressure used to form the articles so that the form to which the mix is pressed will not swell or spring back or otherwise lose its shape when pressure is released. Because the coke or other similar material will not compress and

can be accurately graded in advance the cell size can be determined in advance and produced without particularly skillful handling. This method is easier and more accurate than, for example, a method employing gas bubbles to produce the voids or cells. Furthermore, a mixture employing coke is stable and does not have to be used immediately. Also, when coke is used to form the cells the cell walls tend to be more solid and less porous while by the gas method the cell walls tend to be porous due to minute gas bubbles contained therein.

It will be understood that the above description is not intended to limit the scope of the invention herein but that the invention may be otherwise practiced or embodied without departing from the scope of the claims.

We claim:

1. A mix for making abrasive articles which contains granular abrasive material, bond, and granulated coke.

2. A mix for making abrasive articles which comprises granular abrasive material and granulated coke having an average particle size at least as great as that of the abrasive material.

3. A mix for making abrasive articles which comprises granular abrasive material and granulated coke having an average particle size smaller than that of the abrasive material.

4. A mix for making abrasive articles which consists of granular abrasive material, a vitreous bond, a temporary bond, water, and granulated coke.

5. A mix for making abrasive articles which comprises granular abrasive material and granulated coke having an average particle size greater than that of the abrasive material.

6. In the process of making a bonded abrasive article the steps of adding to the mix granulated coke, pressing the mixture to the desired shape, and effecting removal of the coke granules by firing the shaped article.

7. The process of making a bonded abrasive article which comprises intimately mixing granular abrasive material, suitable bonding material, and granulated coke having an average particle size at least equal to that of the abrasive material, pressing the mixture to the desired shape, and firing the same to burn away the coke granules and vitrify the bond.

8. The process of making a bonded abrasive article which comprises intimately mixing granular abrasive material, suitable bonding material, and granulated coke, having an average particle size several times as great as that of the abrasive material, pressing the mixture to the desired shape, and firing the same to burn away the said oxidizable material and vitrify the bond.

9. The process of making a bonded abrasive article which comprises intimately mixing granular abrasive material, suitable bonding material, and granulated coke having an average particle size smaller than that of the abrasive material, pressing the mixture to the desired shape, and firing the same to burn away the said granulated coke and vitrify the bond.

CHARLES E. WOODDELL,  
JOHN F. BARNES.